

Aug. 3, 1926.

1,594,994

W. A. BONE

TREATMENT OF CERTAIN FUELS TO IMPROVE THEIR CALORIFIC VALUE

Filed July 5, 1919



Inventor  
William A. Bone

By *James L. Morris*  
Attorney

Patented Aug. 3, 1926.

1,594,994

# UNITED STATES PATENT OFFICE.

WILLIAM ARTHUR BONE, OF LONDON, ENGLAND.

## TREATMENT OF CERTAIN FUELS TO IMPROVE THEIR CALORIFIC VALUE.

Application filed July 5, 1919, Serial No. 308,812, and in Great Britain July 30, 1918.

I have discovered that when brown coals and lignites, which have been completely freed from mechanically held water by drying them at temperatures below 110° C., are 5 heated to higher temperatures which are below that at which destructive distillation begins, they undergo a chemical change that begins to be important at temperatures between 250° C. and 400° C. This change is 10 characterized by evolution of water and carbon dioxide, together with a small quantity of carbon monoxide, as substantially the only fluid products; that is to say, the change has nothing whatever in common 15 with what would ordinarily be termed destructive distillation, inasmuch as it is unaccompanied by any evolution of hydrogen, 20 methane or condensable hydrocarbon vapours. Moreover, unlike a destructive distillation, it does not involve any break-down 25 or disruption of the cyclic complex of carbon rings with side chains, which undoubtedly constitutes the main part of the coal substance. The ratio CO<sub>2</sub>:H<sub>2</sub>O in the gases evolved when the dried lignite or brown coal is heated at the aforesaid temperature is usually approximately 1 1 mol. : 2 mols. This indicates that the change consists in an internal condensation of the cyclic complexes of which the coal substance is now 30 generally admitted to consist. The character of such condensation may be symbolized as follows:— 35



35 The technically important result of this chemical change is that it is accompanied by a valuable increase in the calorific value of the fuel. 65

40 My invention is based on the foregoing discovery and consists in heating brown coal or lignite at temperatures between 250°—400° C. until evolution of gases and water vapours ceases, for the purpose of enhancing the calorific value of the material. 70

45 Since the temperature in question does not exceed 400° C. and in the case of some lignites is not above 375° C., the operation or operations necessary for raising the grade of such fuels according to this invention is 75 50 or are of comparatively low cost. The material may be treated in externally heated retorts or chambers by any known continuous or intermittent procedure; but inasmuch as the vapours and gases expelled or 80 produced by the heating are of comparatively little value, it is economical to use internal heating, that is to say, to pass hot vapours or gases through the retort or chamber containing the material, particularly as the 85 temperature required is generally below that of flue gases or like waste gases from boiler 90

furnaces, gas retort settings or the like. Such gases are applicable, provided that they are chemically inert, or substantially so, towards the material at the said temperature, or that their content of reactive oxygen is low enough to avoid exothermic oxidation sufficiently vigorous to raise the temperature of the material above the desired limit. For this reason air alone is seldom applicable when the process is conducted as a single operation. Sometimes, however, it is profitable first to expose the material to heated air at a temperature below that at which exothermic oxidation becomes vigorous, and then to substitute heated gas or vapour sufficiently free from constituents which can react with the material at the higher temperature to which it is heated. In any case the operation of heating the material by hot gases or vapours may be on the counter-current principle, and whatever the mode of heating it may be conducted in more than one stage. 85

The invention may be illustrated by reference to the effect of the process on the Morwell brown coal from Victoria, Australia. This material contains 48 per cent

of water and 52 per cent of coal substance (including ash 4 per cent). Its calorific value is only 5853 B. t. u. per lb. When heated at 105° C. it loses the aforesaid water and then has a calorific value 10,060 B.t.u. per lb.

On continuing to heat the dried material so as to raise its temperature gradually above 105° C. certain chemical changes occur 10 in the coal substance at temperatures between 250° C. and 375° C. whereby more water is expelled together with a small quantity of non-inflammable gas composed chiefly of carbon dioxide. Oil first appears 15 as a product of the heating when the temperature is about 380° C.

Hence the preferable mode of applying the present process to this brown coal consists in heating the coal at a temperature 20 about 375° C. until elimination of water and gases at that temperature has substantially ceased. In this manner 100 parts by weight of the coal dried at 105° C. yield 88 parts of a coal the calorific value of which 25 is 11,460 B. t. u. per lb.

From the foregoing data it may be calculated that 100 parts by weight of the raw coal, 52 parts of the dried coal and 45.75 parts of the treated coal have the same heating value. It follows that the potential 30 energy of the raw coal can be concentrated by this process before transport.

As already stated the heating operation may be conducted in any suitable manner, 35 but preferably by passing hot products of combustion through a column or layer of the fuel, whether vertical, horizontal or inclined. I have found that boiler flue gases having a temperature of 400° C. and containing 10-12.5 per cent. of CO<sub>2</sub>, when passed over the raw coal in question, contain sufficient heat to dry the fuel and to raise its temperature to 375° C. without any danger of exothermic oxidation sufficiently vigorous to raise the temperature of 40 the material higher than this; that is to say without danger of ignition of the coal. This is also true if the gases be passed over the coal which has been dried (at 105°) as a 45 separate operation, but not, in any case, if the content of CO<sub>2</sub> in the gases falls much below 10 per cent. Since, in a properly fired boiler (which may consume the coal in question after it has been treated by the 50 process) it is easy to obtain flue gases containing 10 per cent of CO<sub>2</sub> and to let down the temperature of these gases (if necessary) by means of an economizer, or otherwise, to 400° C., the process becomes a valuable adjunct to a power station consuming 55 the coal.

Apparatus for heating such fuels in this manner will readily be designed by the chemical engineer.

60 A suitable apparatus for this purpose is

shown in the accompanying drawing which represents a vertical section through the furnace chamber *a* of a water-tube boiler having a well known mechanical stoker *b*. As usual, the furnace gases pass from the chamber *a* to the chimney through a port *h*, controlled by a suitable damper, and thence through an uptake *c*. In this uptake is contained a chute *d* down which brown coal is fed to the stoker *b*.

This chute, together with a baffle *i* arranged in the uptake, divides the uptake into an upper and lower compartment. The chute is continued outside the uptake by an upper extension *e* and a lower extension *f*.

That part of the chute which is within the uptake is constructed of bars *d'* which preferably extend transversely of the uptake so that the gases can pass freely between said bars.

The brown coal passes from the chute *d* into the hopper *g* of the mechanical stoker, at substantially the same rate at which the stoker feeds the fuel to the furnace. Thus the chute *d* constitutes a partition in the uptake through which the furnace gases, or a portion thereof, which enter the uptake through the port *h* must pass twice on their way to the chimney, the baffle *i* compelling this course.

For the better regulation of the temperature to which the brown coal is heated, there is a second damper-controlled port *k* for passage of furnace gases into the uptake, above the baffle *i*, so that any desired proportion of the gases, determined by controlling the dampers in the ports *h* and *k*, may pass to the chimney without passing through the chute.

What has been said with reference to the 105 Morwell brown coal applies to other fuels of the kind here in question, it being understood that the composition, calorific values and temperature of heating vary with each particular fuel. For instance, certain 110 Italian lignites (containing 21.5 per cent. of water) when dried at 105° C. and heated, first yield oils at 310-320° C. and when heated at 300° C. give 88 parts by weight of concentrated fuel per 100 parts of dry fuel; the calorific value of this concentrated fuel is 9698 B. t. u. per lb. as compared with 8278 B.t.u. per lb. for the dried fuel.

Having thus described the nature of the 115 said invention and the best means I know of carrying the same into practical effect, I claim:—

1. A process whereby the calorific value of brown coals or lignites may be increased, which consists in relatively moving in contact with each other the coal or lignites and flue gases having a temperature between 250° C., and 400° C., until evolution of gases and water vapour from the material ceases.

2. A process whereby the calorific value of brown coals or lignites may be increased which consists in relatively moving in contact with each other the coal or lignites and flue gases containing not less than 10 per cent. of carbon dioxide and having a temperature between 250° C. and 400° C. until evolution of gases and water vapour from the material ceases.
- 10 3. A process whereby the calorific value of brown coals or lignites may be increased, which consists in relatively moving in contact with each other the lignite or coal and the flue gases formed by combustion of said lignite or coal, the carbon dioxide content of which flue gases is not below 10 percent, and at a temperature not exceeding 400° C.
- 15 until water vapor and gases cease to evolve from the coal or lignite.
4. A process for increasing the calorific value of brown coals or lignites by causing the evolution of water vapor and carbon dioxide substantially free from hydrocarbons and uncombined hydrogen, which consists in heating the material at such a rate and at a temperature not substantially in excess of 400° C. that such evolution takes place, and continuing the heating of the material at a temperature not substantially above 400° C. until such evolution ceases. 30
- In testimony whereof I have signed my name to this specification.

WILLIAM ARTHUR BONE.